

as will be apparent in the following claims, until well impregnated with the preservative, and then to boil the wood in a solution of sulfur and resin until the wood is rendered substantially non-absorbent and to increase its electrical insulating qualities.

# UNITED STATES PATENT OFFICE.

WILLIAM WEIMAR, OF APPLETON, WISCONSIN.

## PROCESS FOR TREATMENT OF FIBROUS MATERIAL.

1,313,437.

Specification of Letters Patent. Patented Aug. 19, 1919.

No Drawing.

Application filed October 22, 1917. Serial No. 197,893.

To all whom it may concern:

Be it known that I, WILLIAM WEIMAR, a citizen of the United States, residing at Appleton, in the county of Outagamie and 5 State of Wisconsin, have invented certain new and useful Improvements in Processes for Treatment of Fibrous Material, of which the following is a specification.

My invention relates to processes for treatment of fibrous material such as wood, and the like.

One of the objects of my invention is to provide a process for the treatment of wood, wood pulp, fiber board, card-board and other 15 fibrous substances or material whereby to render them water, weather, and acid proof and to increase their insulating and other desirable qualities.

In carrying my invention into effect, I 20 first subject the material to a preservative, such as a saturated solution of sodium chlorid and then fill the pores of the material with a filler possessing decay and electric current resisting substance such as sulfur and 25 the common resin of commerce. When relatively soft and porous wood has been properly treated by my process, the product has an enhanced value and possesses a much higher specific gravity, having the qualities 30 and appearance of the more expensive wood and it is equally well adapted as ebony, for use in making brush and mirror backs, piano keys, toilet sets, keys for other musical instruments, such as violins, banjos, guitars 35 and the like. Owing to its relatively high current resisting or insulating qualities, it may be substituted in many situations for hard rubber or other more expensive insulating materials in the construction of electrical 40 apparatus and instruments.

Specifically, the desideratum is to drive out of the pores of the wood any resident content and then to coat the pores with a liquid preservative and finally to fill them 45 with the preserving and insulating compound.

Wood bodies or pieces of suitable size are immersed in a preferably saturated solution of wood preservative, such for instance as 50 sodium chlorid. The solution is maintained hot and the wood should remain in the solution preferably, for 24 hours or until the solution has thoroughly permeated the wood body. The wood may first have been kiln- 55 dried or green wood may be used if the preserving solution is heated to the boiling

point, this will drive out the sap and allow the entrance of the saline solution. From this solution the wood is removed and dried or allowed to dry, superficially. It is then 60 placed in a vat or other suitable receptacle containing boiling sulfur and resin. I have found that sufficient sulfur should be used to submerge the wood and that very good results may be obtained when the resin is 65 about one per cent. in weight of the sulfur or ninety-nine per cent. of sulfur and one per cent. of resin may be satisfactorily used.

The fibrous material should be maintained in this boiling solution until it assumes the 70 desired color and weight. The time required for this immersion depends to some extent upon the character of the body or material operated upon. For example, in the treatment of wood the time that it shall remain in 75 the boiling sulfur-resin solution varies from 3 to 7 days.

After the substance has been cooked in the sulfur solution, for the requisite period of time, it is taken out and rapidly cooled. 80 This may conveniently be done by immersing it in cold water. This has the effect of converting the sulfur into a plastic state rendering the treated body less brittle than it would otherwise be if allowed to cool 85 slowly.

The word resin, as used in the claims, refers to the common resin of commerce, a by-product in the manufacture of turpentine from the exudation of trees or plants of the 90 conifer family.

While I have described my process in minute detail it will be manifest that changes in the specific manner of carrying my invention into effect may be made within the scope 95 of the appended claims.

Having described my invention, what I claim is:

1. The process of treating fibrous material such as wood or the like which consists in 100 impregnating the material with a solution of sodium chlorid, or the like; then boiling it in a solution of sulfur and resin, then cooling it.

2. The process of treating fibrous material 105 to render it substantially non-absorbent and to increase its electrical insulating qualities which consists in immersing it in a hot saturated solution of sodium chlorid for a protracted period of time; then removing it 110 from the solution and drying it; then placing it in a solution of sulfur and resin main-

tained at temperature sufficient to boil the sulfur until the pores are sufficiently filled; then removing the material from the sulfur bath and immediately cooling it by application of water.

3. The process for treatment of fibrous material, such as wood or the like, which consists in dehydrating the material; immersing it in a hot saturated solution of sodium chlorid; then superficially drying the material; then submerging said material in a hot solution of sulfur and resin, then cooling it.

4. The process for treating of fibrous material to render it substantially non-absorbent and non-conductive, such as wood or the

like, which consists in immersing it in a hot saturated solution of sodium chlorid; removing it from the solution and superficially drying it; then cooking it in a solution of sulfur and resin with the sulfur maintained at its boiling point; then removing it from the latter solution and quickly cooling it.

In testimony whereof I hereunto set my hand in the presence of two subscribing witnesses.

WILLIAM WEIMAR.

In the presence of—

MOLLIE E. PFEFFER,  
C. G. CANNON.